

## 1

3,318,423

## VEHICLE BRAKE PART

Walter Dunki, Zurich, Switzerland, assignor to Escher Wyss Aktiengesellschaft, Zurich, Switzerland, a corporation of Switzerland

No Drawing. Filed Sept. 8, 1964, Ser. No. 396,275  
 Claims priority, application Switzerland, Oct. 10, 1963,  
 12,453/63

11 Claims. (Cl. 188—251)

This invention relates to a vehicle brake part subjected to stress by sliding friction.

Vehicle brake parts, for example brake shoes, subjected to stress by sliding friction, have heretofore usually been made of grey cast iron, to some extent of cast steel, sometimes low-alloy highly heat-treated cast steel, sometimes with somewhat modified composition.

The brake-shoe specification of a well-known railway company is, for example, as follows:

|            | Percent  | 20 |
|------------|----------|----|
| Carbon     | 3 to 3.3 |    |
| Graphite   | 2 to 2.5 |    |
| Silicon    | 1.8      |    |
| Phosphorus | ≤0.8     |    |
| Sulphur    | ≤0.15    |    |
| Manganese  | 0.45     |    |

With vehicle brake parts subjected to stress by sliding friction it is intended to obtain a good braking effect, and also the wheels or wheel rims should be protected as much as possible. In vehicle brake parts subjected to stress, considerable wear is an undesirable occurrence. The wear dust consists partly of reddish-brown rust, which can be very troublesome. As the result of wear, the brake parts have always to be replaced after a comparatively short service period. Attempts have already been made, inter alia by varying the alloy composition, to effect a reduction in wear. Thus, for example, the phosphorus content has been increased, in some cases up to 1.5%, or small additions of chromium up to 1.5%, and of molybdenum or vanadium up to a few tenths of a percent, have been made. Wear has thus been reduced somewhat, but the braking effect was impaired, and to some extent, the braking surface of the wheel or tyre has been damaged. Heretofore, it has not been possible to employ successfully brake shoes of such cast iron, or they have not been accepted in practice.

This invention now consists in that a vehicle brake part subjected to stress by sliding friction is made of a high-carbon, austenitic iron alloy having a proportion of free carbon.

It has been surprisingly found that brake parts of the aforesaid material have excellent service properties. This was not to be expected, since such a material costs several times more than, for example, the material used heretofore for brake shoes, and it is only possible because unexpected braking properties are obtained by means of such austenitic material, namely very low wear coupled with the best braking effect and maximum protection, for example, also of wheels and tyres. By this means, the resulting life is increased by several times, so that despite the high cost, the result is a considerable economic advantage. Austenitic structure of the material is preferably obtained by a nickel addition of between 10% and 25%. Some of the nickel may also be replaced by manganese in an amount of between 0.5% and 7%.

In addition to the two austenite formers—nickel and manganese—it has been found advantageous to add also a certain copper content, which dissolves in the austenite, and may amount to from about 0.5 to 4%. It is furthermore advantageous to imbed in the groundmass, in addition to austenite, hard constituents, such as carbides, phos-

## 2

phides and so forth. The following come into consideration for this purpose: iron carbide and carbides of carbide-forming elements such as chromium, molybdenum, vanadium, and titanium, as well as phosphorus. The addition of chromium may amount to about 0.5 to 3%, that of molybdenum, vanadium and titanium each to about 0.1 to 1% and that of phosphorus to about 0.6 to 1.5%.

Part of the carbon is present in the alloy in the free form as lamellar or spheroidal graphite. The latter form of graphite is obtained by treatment with the addition of magnesium or cerium or both. Such an austenitic cast iron for brake parts has, for example, the following typical analysis:

|            | Percent |
|------------|---------|
| Carbon     | 2.8     |
| Silicon    | 2.3     |
| Phosphorus | 0.6     |
| Sulphur    | 0.06    |
| Nickel     | 19      |
| Manganese  | 1.5     |
| Copper     | 2.0     |
| Chromium   | 0.1     |

The material may also be subjected to a heat treatment, for example by annealing at a temperature between 800° C. and 1000° C. with accelerated or unaccelerated cooling.

A further advantage of the austenitic cast iron for brake parts is provided by its much higher strength and deformation properties compared with grey cast iron; these properties for example, make it possible to dispense with the steel lining necessary in the case of grey cast iron shoes.

The following comparison provides information in this connection:

|                                               | Ordinary cast iron | Austenitic cast iron |
|-----------------------------------------------|--------------------|----------------------|
| Tensile strength, kg./mm. <sup>2</sup>        | 15 to 20           | >35                  |
| Elongation, percent                           | <1                 | 10 to 40             |
| Notch impact toughness, kgm./cm. <sup>2</sup> | <0.3               | >3                   |
| Brinell hardness, kg./mm. <sup>2</sup>        | 180 to 250         | 170 to 60            |

It must also be pointed out that austenitic cast iron for brake parts practically does not rust or is almost rustless.

The invention may be used not only for brake shoes, acting on the wheel rims of railway vehicles, but also for other brake parts, which are subjected to stress by sliding friction, for example for brake discs.

What is claimed is:

1. A vehicle frictional brake part subjected to stress by sliding friction, consisting of a high-carbon, austenitic iron alloy having a proportion of free carbon.
2. A brake part according to claim 1, in which the austenitic structure comprises a nickel addition of 10% to 25%.
3. A brake part according to claim 2, in which for austenite formation, part of the nickel has been replaced by manganese from 0.5% to 7%.
4. A brake part according to claim 1, in which the material contains 0.5 to 4% copper.
5. A brake part according to claim 1, in which the material contains 0.5 to 3% chromium.
6. A brake part according to claim 1, in which the material also contains addition of 0.1 to 1% of at least one of the materials molybdenum, vanadium and titanium.
7. A brake part according to claim 1, in which the material contains 0.6 to 1.5% phosphorus.
8. A brake part according to claim 1, in which the carbon content is present partly in carbide form and partly as free carbon (lamellae graphite).

9. A brake part according to claim 1, in which the free carbon is present in spheroidal form.

10. A brake part according to claim 1, in which the material is subjected to a heat treatment by annealing between 800° C. and 1000° C.

11. A vehicle frictional brake part subjected to stress by sliding friction consisting of a high-carbon austenitic iron alloy having a proportion of free carbon, comprising the components nickel, carbon, silicon, copper, manganese, phosphorus, chromium, sulphur substantially in the proportions 19%, 2.8%, 2.3%, 2.0%, 1.5%, 0.6%, 0.1%, 0.06%, respectively.

## References Cited by the Examiner

## UNITED STATES PATENTS

|           |        |                  |       |        |
|-----------|--------|------------------|-------|--------|
| 2,842,437 | 7/1958 | Guenzi           | ----- | 75—125 |
| 3,055,755 | 9/1962 | Schelleng et al. | ----- | 75—123 |

## 5 FOREIGN PATENTS

807,302 10/1936 France.

HYLAND BIZOT, Primary Examiner.

16 DAVID L. RECK, Examiner.

P. WEINSTEIN, Assistant Examiner.